

# UNITED STATES PATENT OFFICE.

PHILIP POORE, OF LONDON, ENGLAND.

## DISTILLATION OF WOOD, WOODY FIBER, AND SIMILAR CARBONACEOUS SUBSTANCES.

1,397,181.

Specification of Letters Patent.

Patented Nov. 15, 1921.

No Drawing.

Application filed July 7, 1918. Serial No. 309,121.

*To all whom it may concern:*

Be it known that I, PHILIP POORE, a subject of the King of Great Britain and Ireland, residing at 1/4 Paternoster Row, London, E. C., England, engineer, have invented certain new and useful Improvements Relating to the Distillation of Wood, Woody Fiber, and Similar Carbonaceous Substances, of which the following is a specification.

10 This invention relates to the destructive distillation of wood, woody fiber and similar carbonaceous substances and has for its object to carry on the distillation under such conditions as to secure a high yield of acetic acid, wood naphtha, or other distillation products.

According to the invention I admit steam at a temperature of from about 180° C. to about 270° C. into the retort throughout the 20 active period of distillation or for a period extending over the time during which the exothermic reaction takes place and which generally commences on the charge reaching a temperature of about 270° C., and I render the application of heat throughout the charge substantially uniform. For this purpose the distillation may be effected in retorts which are rotated continuously or periodically during the distillation as described 30 in the specification filed pursuant to a co-pending application, the petition being dated the 20th January, 1919.

In carrying the invention into effect in the use of stationary cylindrical retorts into 35 which the superheated steam is admitted at the bottom of the retort from a perforated pipe extending the length of the retort as described in the specification of the prior application made by me No. 239237 40 dated 10th June, 1918, I have found that if the superheated steam on passing into the retort has a temperature of from 180° C. to 270° C. a very high yield of acetic acid and other distillation products will be secured 45 under the conditions there prevailing. In the distillation of pine wood and hirch wood, I have found if the steam admitted to the retort has a temperature of from 210° to 225° the highest yield of acetic acid and other 50 distillation products will be secured. It will, however, be understood that in such a case the wood or other carbonaceous material is first cut up into pieces and dried so as to reduce its content of moisture to such an extent as conveniently practicable, for example to about five or ten per cent. of moisture

and that the admission of superheated steam into the retort is delayed until such time that the evolution of the residual content of moisture in the charge is completed and the 60 charge has acquired a temperature of over 100° C. so that thus in no part of the period of distillation may the steam fall below the condensing point. In the use of cylindrical retorts, I prefer, however, to provide the 65 retort of a large size and so mounted as to be capable of periodic or continuous rotation as for example once in four minutes.

Such a retort is described in the specification of the co-pending application aforesaid dated the 20th January, 1919. In the use of such retort, the application of heat to the charge and the distribution of steam therethrough at a temperature within the range hereinbefore specified is rendered uniform and by distillation under these conditions I have secured higher yields of the distillation products than when the stationary retort of the first modification is employed.

From the foregoing it will be understood that by admitting steam within the range of temperature indicated a relatively high yield of the distillation products is secured and that with a view still further to improve the yield where using a cylindrical retort it is preferable to cause its rotation for the purposes described. By such means the total yield of the distillation products is increased.

In the use of the cylindrical retort whether stationary or rotary I prefer to provide a centrally disposed and perforated outlet pipe which when the retort is arranged to rotate permits of the movement of the charge 95 in the retort in the manner described in the specification of the co-pending application aforesaid dated the 20th January, 1919.

I claim:

1. A method of increasing the yield of 100 acetic acid, wood naphtha, or other distillation products in the destructive distillation of wood, woody fiber and similar carbonaceous substances, consisting in subjecting the charge to distillation at a gradually 105 increasing temperature by the uniform external application of heat to the retort within which the distillation is effected, and admitting steam into the retort at a substantially constant and relatively low temperature 110 during the active period of distillation, substantially as described.

2. A method of increasing the yield of acetic acid, wood naphtha, or other distillation products in the destructive distillation of wood, woody fiber and similar carbonaceous substances, consisting in subjecting the charge to distillation at a gradually increasing temperature by the external application of heat to the retort within which the distillation is effected, and admitting steam 10 into the retort at a substantially constant temperature between from about 180° C. to about 270° C. during the active period of distillation, substantially as described.

3. A method of increasing the yield of acetic acid, wood naphtha or other distillation products in the destructive distillation of wood, woody fiber and similar carbonaceous substances, consisting in applying heat externally to the retort to effect the 20 distillation and in the admission of steam into the retort at a temperature between from about 180° C. to about 270° C. for the purposes and substantially as described.

4. A method of increasing the yield of acetic acid, wood naphtha or other distilla- 25

tion products in the destructive distillation of wood, woody fiber and similar carbonaceous substances, consisting in applying heat externally to the retort to effect the distillation and in the admission of steam into the 30 retort at a temperature between from about 180° C. to about 270° C. throughout the active period of distillation and subjecting the retort to rotation during the distillation, for the purposes and substantially as de- 35 scribed.

5. A method of increasing the yield of acetic acid, wood naphtha or other distillation products in the destructive distillation of wood, woody fiber and similar carbonaceous substances, consisting in applying heat externally to the retort to effect the distillation and in the admission of steam into the 40 retort at a temperature between from about 180° C. to about 270° C. for a period extending over the time during which the exothermic reaction takes place, substantially as described. 45

PHILIP POORE.